

1,477,516

Dec. 11, 1923.

T. W. MILLER

GOLF BALL

Filed Oct. 5, 1923

GUTTA PERCHA  
OR  
BALATA



Inventor  
Thomas W. Miller  
by Percy B. Hills  
Attorney

Patented Dec. 11, 1923.

1,477,516

# UNITED STATES PATENT OFFICE.

THOMAS W. MILLER, OF ASHLAND, OHIO.

## GOLF BALL.

Application filed October 5, 1923. Serial No. 666,842.

To all whom it may concern:

Be it known that I, THOMAS W. MILLER, a citizen of the United States, residing at Ashland, county of Ashland, State of Ohio, have invented certain new and useful Improvements in Golf Balls, of which the following is a specification.

My invention relates to golf balls, and compositions therefor, and is a continuation in part of an application for golf ball compositions, filed by me May 18, 1922, Serial No. 561,943, and has for its objects, first, economy in the manufacture, at the same time producing a ball which will have to a very considerable degree all of the desirable qualities of golf balls now on the market, and, secondly, to eliminate the liability of cutting the ball if topped or struck with the edge of the driving club when in play.

20 In the accompanying drawing:

The figure is an enlarged sectional view of my improved golf ball.

In carrying out my invention, I first prepare a rubber stock 1 from material suitable to produce a composition of the desired gravity, density, resiliency and resistance to cutting, as hereinafter set forth. After milling and preparing said stock, it is cut into sections each of substantially the weight 25 of a finished golf ball, and each of said sections then is placed in registering molds and heated and vulcanized under pressure. Said molds are provided either with projections or depressions to produce the dimple or 30 bramble effect as desired, so that the ball so compressed and vulcanized as it comes from the mold will have the true exterior design of the finished ball, and also will have the same diameter less the thickness of the cover.

40 After vulcanization and removal from said mold any selvage or overflow at the line of mold registration is removed, and the ball then is cleaned from all undesirable substances by boiling in a suitable solution.

45 The ball then is placed on a suitable dipping board and dipped in a solution of balata or gutta-percha, to which has been added pigments or fillers to give the finished ball the desired color. The coating 2 of balata or 50 gutta-percha so applied will conform to the exterior configuration of the pre-formed ball, and if desired a finishing coat of suitable varnish or lacquer may be applied thereto by dipping.

55 The object of applying the dipped cover

2 is to provide a comparatively hard unyielding surface, the variation of which in thickness affects the distance flight of the ball, and also its rebounding properties after striking the ground. A further object is to provide the desired color for the finished ball.

From the above description, it will be understood that the unfinished ball as it comes from the mold will have the true design of 65 the finished ball and substantially its diameter, as in ordinary practice the thickness of the cover will be negligible. As it is desirable that the finished ball have an uneven surface, either of depressed or raised design and shown in the drawing as dimples 3, commonly known as the dimple and bramble designs, and that of a sharp pattern, and as it may be found desirable to apply a cover of a thickness which will destroy the 70 sharp outline of the surface design, the ball after the dipped cover has been applied again can be placed in a mold of a proper size and design, and by applying heat under pressure, the surface design will be brought 75 out more sharply.

A composition which will produce a ball closely approximating the standard ball in its functions embodies the following ingredients and approximate proportions:

|            | Pounds.            |
|------------|--------------------|
| Rubber     | 32                 |
| Glue       | 18                 |
| Zinc oxide | 10 $\frac{1}{2}$   |
| Sulphur    | 2 $\frac{1}{2}$ 90 |

It has been found that a composition of the above formula when vulcanized will resist cutting to a very high degree, and this result is accomplished primarily through the 95 use of the rubber and glue ingredients. It will be understood, however, that I do not limit myself to these proportions, as the glue and rubber content may be varied somewhat, and certain fillers, such as aluminum 100 flake and asbestos added, with satisfactory results.

While I prefer to form the ball solid, it will be understood that the same may be formed with a hollow center.

Having thus fully described my invention, what I claim as new and desire to secure by Letters Patent, is:

1. A golf ball, comprising a homogeneous body portion embodying as a composition,

- rubber, glue, a vulcanizing agent, and a filler in such proportions as will approximate the standard ball in size and weight, said body portion being formed and vulcanized to the 5 surface configuration of the finished ball, and a thin cover or finishing coat which conforms to said surface configuration.
2. A golf ball, comprising a homogeneous body portion embodying as a composition, 10 rubber, glue, a vulcanizing agent, and a filler in such proportions as will approximate the standard ball in size and weight, said body portion being formed and vulcanized to the surface configuration of the 15 finished ball, and a thin cover or finishing coat which conforms to said surface configuration.
3. A golf ball, comprising a homogeneous body portion embodying as a composition, 20 rubber, glue, a vulcanizing agent, and a filler in such proportions as will approximate the standard ball in size and weight, said body portion being formed and vulcanized to the surface configuration of the 25 finished ball, and a thin cover or finishing coat containing a pigment.

which conforms to said surface configuration.

4. A vulcanizable composition for golf balls, comprising rubber, glue, a filler, and 30 a vulcanizing agent, in such proportions as, when formed into a ball substantially 1.62" in diameter, will weigh, with the finished coating or covering, approximately 1.62 ounces.

35 5. A vulcanizable composition for golf balls, comprising rubber, glue, a filler, and a vulcanizing agent, in such proportions as, when formed into a ball substantially 1.62" in diameter, will weigh, with the finished 40 coating or covering, approximately 1.62 ounces, and possessing a proper resiliency and a high resistance to cutting.

6. A vulcanizable composition for golf balls, comprising rubber approximately 32 45 parts, glue approximately 18 parts, zinc oxide approximately 10.5 parts, and sulphur approximately 2.5 parts.

In testimony whereof I hereunto affix my signature.

THOMAS W. MILLER